

## UNITED STATES PATENT OFFICE

2,004,473

## PRODUCTION OF LEATHER

George R. Pensel, Amsterdam, N. Y.

No Drawing. Application April 21, 1933,  
Serial No. 667,306

26 Claims. (Cl. 149—3)

This invention relates to the production of leather from hides or skins, and more particularly to tanning processes in which the hides or skins are subjected to certain novel treatment prior to the actual tanning thereof.

This preliminary treatment has special application to chrome tanning, although it may be used to great advantage in other types of tanning processes, including those in which formaldehyde or other aldehydes are employed, in vegetable tanning processes or the so-called bark tannages, and also in oil tannages.

The present application is a continuation in part of my prior application Ser. No. 541,122, filed May 29, 1931, and has for its general object the provision of novel and improved methods and compositions for effecting the tanning processes to which reference has been made.

As is generally well known, before being tanned or converted into leather, hides and skins are subjected to certain preliminary processes including the steps of dehairing, liming, bating and beaming. Upon removal from the beamhouse, the skins are placed in a pickling bath which almost invariably comprises a solution of sulphuric acid and common salt. Although pickling solutions are used for numerous reasons, the chief purpose of the pickling process is to preserve the unhaired skins so that they may be kept for an indefinite period before tanning, as for example, in the case of skins obtained from abroad. Such skins are received in a semi-wet state due to the adhering pickling solution, so that, for example, a dozen skins of a certain kind and size that weigh approximately twenty or twenty-one pounds in the pickle, weigh only about eight pounds when dry. These pickled skins are quite strongly acid and generally have a pH value of from 1.9 to 2.2.

In previous vegetable tanning processes, these strongly acid skins have been subjected to a neutralizing or depickling process by the use of an alkali such as borax or sodium bicarbonate so as to bring the hydrogen ion concentration of the skins to about pH 3 or 4. In the case of aldehyde tannage the range of pH values prior to tanning have run from 7 to 12, but the pH numbers have generally been brought down to the neighborhood of 7 to 9 during the actual aldehyde tanning steps. It is noteworthy that in prior processes of chrome tanning, it has not been considered necessary to depickle the skins.

My novel and particularly effective preliminary treatment is applied to the skins after the pickling step. Generally in the case of imported skins which are pickled abroad, the treatment

is applied directly to the skins as received and prior to the actual tannage. One exception to this procedure may occur in cases in which the skins are degreased. This preliminary treatment comprises what might be termed a "re-pickling" step or, in other words, a substitution process by which the strong acid pickle is replaced by a weaker acid, preferably of an organic nature, and whereby the pH number is raised from about 2.0 to the neighborhood of 5.0. This "re-pickling" has been found beneficial in all types of tanning whether aldehyde, bark or chrome, but more especially in the last named type in connection with which most remarkable results have been obtained. Formerly, successful chrome tannage processes involved soaking the skins in the tan liquor all day with constant additions of material and supervision, and the most rapid chrome tanning previously attained has taken from five to ten hours. But it has been found that by pursuing the process involving the principles of the present invention the skins may be chrome tanned so as to stand the familiar boiling test in about fifteen minutes. So-called short tanning processes to which reference has been made, were dependent upon high concentrations of basic chromium sulphate solutions and neutralization with alkalies. The chromium in my method is "fixed" without the use of alkalies.

The complete theory and explanation of the present invention is not thoroughly understood in all its details, but it is well recognized that the fundamental operations in the complete tannage process are interdependent, and therefore this invention comprises not only the novel preliminary acid substitution or "re-pickling" but the novel combination of this treatment with the subsequent tanning process.

In its preferred embodiment, my new method may be briefly described as involving the substitution of acetic or other relatively weak organic acid for the sulphuric acid in the pickled skins, whereby among other effects, the pH number of the batch is raised to the neighborhood of 4.8-6.0; controlling the temperatures and concentration of the various salts, acids and bases involved within certain limits to better effectuate the process; and then tanning the skins by certain rapid but effective steps to be described in detail in the specification to follow. In the chrome tannage to which the present invention is most particularly adaptable, the pH numbers of the tannage baths are also maintained at values in the neighborhood of 5.0. In the case

of the formaldehyde tannage the pH number of the bath after depickling may be as high as 5.5, and during early tanning stages about 7.4, where it is maintained as closely as possible by the addition of suitable agents.

In order to present a complete disclosure whereby the invention may be practiced by one skilled in the art, the following detailed descriptions are submitted merely by way of example, 10 the invention not being limited to the detailed steps and quantities named except within the scope of the subjoined claims.

A formaldehyde tannage has been successfully effected as follows: 468 pounds of skins (pickled 15 weight) were floated in a revolving drum in about 100 gallons of the following solution: About 150 pounds of Glauber's salt (for suede leather about 100 pounds and for strong grain leather about 200 pounds); 44 pounds of sodium acetate (9% 20 of the pickled weight of the skins); 6.1 pounds of 84% acetic acid (1.3% pickled weight of skins). The drum containing the skins and this solution was revolved for about 30 minutes at about 80° F. The pH number of the bath was at that 25 time about 5.1.

About 16 pounds, 6 ounces of borax was dissolved in about 6 gallons of boiling water, and there was added 15 gallons of cold water and about .50 pounds of Glauber's salt which reduced 30 the temperature of the solution to about 80° F. The solution thus prepared was added to the drum and the latter was revolved for about 30 minutes. The pH number was then in the neighborhood of 5.5.

The skins were then "slatted off", or, in other words, drained in a rotating drum having a door with open slots or holes through which most of the liquor in the skins may drain away, and they were ready for the actual tanning process. One 40 hundred gallons of the tanning solution were prepared as follows: 150 pounds Glauber's salt; 20 pounds borax (about 4% of the pickled weight of the skins); 58 pounds (about 12%) of Paratan or formaldehyde tanning compound; about 1.2 45 pounds of 84% acetic acid (0.25% of pickled weight of skins). The drum containing the pickled skins was revolved and this tanning solution was added at a final temperature of 80° F. The drum was revolved for one hour and the pH 50 number was then found to be about 7.4, and the temperature of the bath is raised to about 100° F. There was added about 14 pounds (3%) of a suitable sulphonated oil, the drum was revolved for 10 minutes and the temperature raised to about 55 120° F. Enough borax was added along with the sulphonated oil to insure that there would be no change in the pH number. The drum was then revolved for about 30 minutes at 120° F.; the temperature was raised to 130° F. during another 60 30 minute run; the bath was then run for 30 minutes to 140° F., and was then run for another 30 minute period at 140° F. The pH number was still about 7.4. The skins were then washed until they were reduced to a temperature of about 80° F. 65 It is to be noted that the amount of borax added depends to some extent on the acidity of the original pickle and upon the pH value, in the neighborhood of 7, desired. For so-called doeskins or suede leather, it is necessary to tan at a pH number slightly below 7 in order to keep the skins firm or slightly under-tanned, while in the case of grain leather, it is necessary to tan at a pH value of above 7 in order to obtain a strong grain.

Specific examples of the chrome tannage process are as follows:

I. About 450 pounds of skins containing their absorbed strong acid pickling at about pH 2.1 were run in a revolving drum for about 30 minutes at 90° F. in 100 gallons of a float containing about 150 pounds Glauber's salt at 80° F.; 40.5 pounds sodium acetate (approximately 9% of the pickled weight of the skins); 5.85 pounds acetic acid (1.3% of pickled weight of skins); and water. The pH value of the skins was then about 5.1.

There was then added to the drum 9.0 pounds 10 of borax (approximately 2%) in 25 gallons of water together with enough Glauber's salt to obtain a salt concentration of about 15% (about 150 pounds); the drum was then revolved for about 30 minutes and the pH value was found to still be in the neighborhood of 5.1. The skins were slatted off and were subjected to a chrome tannage as follows:

About 100 gallons of an aqueous solution containing about 84 pounds (10% concentration) 20 of Glauber's salt crystals or 48 pounds (about 6%) of common salt was introduced, the drum was started, and there was added in three feeds about five minutes apart, a 30% (3 pounds per gallon) aqueous solution of basic chromium sulphate. At the end of 15 minutes the chrome solution was practically exhausted and the skins were sufficiently tanned to stand a boil. The pH number after the tanning was about 4.8-5.0.

Finally, the skins are neutralized with a 1% 30 borax solution to a pH number of 5.9 for coat leather and 6.2 for glove leather, using in the latter case 2% borax based on the pickled weight of skins. It is only necessary then to go ahead with the usual process of fat liquoring or re-tanning for special leathers. In order to produce tighter or looser leather, the pH number may be altered slightly in the depickling stages by the use of sodium formate, sodium acetate, sodium lactate, or other salts of organic acids.

II. The following is an example of a chrome tanning process as applied to certain domestic skins. Approximately 450 pounds of pickled skins had a pH number of 1.2. The float was prepared by dissolving 63 pounds common salt 45 (about 13.8% of the pickled weight of the skins), 42 pounds of a neutralizer, preferably sodium acetate (about 9%), and about 5½ pounds of 84% acetic acid (about 1.2%). The skins were run in this float for about 20 minutes and the pH 50 value was determined to be approximately 4.9. Then about 9 pounds 6 ounces of borax (2% of pickled weight) and about 40 pounds of common salt were added to the float and the drum was run for about 20 minutes, whereupon the pH 55 number was found to be 4.9-5.0. The skins were then drained for 40 minutes.

In the actual tanning stage, a solution is prepared by adding 37 pounds of basic chromium sulphate of a basicity of 38 (8% pickled weight) to 12 gallons of water and an equal quantity of common salt in about 75 gallons of water at 80° F. This tanning solution was added to the skins in three feeds, five minutes apart and the run was continued for 10 minutes after the last feed (total tanning time 25 minutes). The pH number of the skins was then at about 4.9-5.0.

Certain of the skins were then removed for suede finishing and others for fleshing. The 70 fleshed skins were then returned to the drum in the amount of 233 pounds. They were washed with water at 80° F. for 15 minutes and heated to 110° F. There was then added 2 pounds 5 ounces of borax (1% weight of skins) in three feeds, five 75

minutes apart, at 110° F. The pH number was found to be 5.1.

The skins were washed for 15 minutes at 110° F. and then about 9½ pounds (4%) of a synthetic tannin in 6 gallons of water at 110° F. was added and the drum was rotated for 20 minutes. The pH value was then about 5.0. This synthetic tannin is made from orthocresol, sulphonated and condensed with formaldehyde; the sulphonated acid being partially neutralized and buffers being used to raise the pH number. The skins were then washed for 15 minutes at 120° F. and the temperature was then raised to 130° F. They were then put through a fat-liquoring process with suitable compounds, such as sulphonated sperm and coconut oils.

It may be noted at this point that instead of using either Glauber's salt or common salt along with the borax in the neutralizing step following the initial weak acid substitution or depickling, a mixture in suitable proportions of both of these salts may be employed. It has been discovered that the use of Glauber's salt gives a greater stretch to the leather which is desirable in some instances, while common salt gives a tighter skin, and it may be advisable in some cases to combine these salts to obtain a medium effect.

The depickling process in the case of bark tannage is the same as for chrome tannage.

It is understood, as has already been stated, that the percentages, quantities, temperatures and other details of the process just described are stated for example only and may be varied within certain limits without departing from the scope of the invention as set forth in the following claims. Furthermore, it will be clearly realized that the particular re-pickling or substitution process described is not to be confused with any previously known neutralizing, bating, or delimiting steps which are taken at quite different stages of the production of leather, and that this step is only to be applied at a point subsequent to the known pickling step and prior to the actual tanning procedure. It will also be understood that the term "tanning" employed in the broad or generic claims refers to any suitable process of tanning or converting the prepared skins into leather.

The tanned skins obtained as the result of pursuing the present invention may be subsequently put through various processes such as fat liquoring, crusting and dyeing, but these processes are not part of the present invention and are not set forth in any detail in the present application.

Having thus described the invention, what is claimed as new and desired to be secured by Letters Patent is:

1. In the process of producing leather from skins, the step of treating the pickled skins with a salt of a soluble organic acid, prior to tanning.
2. In the process of producing leather from skins, the step of treating the pickled skins with a salt of an organic acid together with a quantity of said organic acid itself, prior to tanning.
3. In the process of producing leather from skins, the step of treating the pickled skins with an alkali salt of an organic acid together with a quantity of said organic acid itself, prior to tanning.
4. In the process of producing leather from skins, the step of treating the pickled skins with a soluble salt of a soluble fatty organic acid, prior to tanning.
5. In the process of producing leather from skins which have been pickled in a strong acid,

the step of replacing the strong acid in the skins with acetic acid prior to tanning.

6. In the process of producing leather from skins which have been pickled in a strong acid, the step of raising the pH number of the pickled skins to approximately 5 by the replacement of said strong acid by acetic acid.

7. In the process of producing leather from skins which have been pickled in a strong acid, the steps of raising the pH number of the pickled skins to the neighborhood of 4.8-5.2 by the replacement of said strong acid by a weaker acid, and then adding a small quantity of a neutralizing agent in the presence of a solution of a salt of the group comprising Glauber's salt and sodium chloride.

8. In the process of producing leather from pickled skins, the steps of agitating a quantity of such skins in an aqueous solution of Glauber's salt, sodium acetate and acetic acid, then adding to the bath an aqueous solution of borax and Glauber's salt, and agitating further prior to tanning.

9. In the process of producing leather from pickled skins, the steps of agitating a quantity of such skins in an aqueous solution of Glauber's salt, sodium acetate and acetic acid, then adding to the bath an aqueous solution of borax and common salt, and agitating further prior to tanning.

10. In the process of producing leather from pickled skins, the steps of agitating a quantity of such skins in an aqueous solution of Glauber's salt, sodium acetate and acetic acid, then adding to the bath an aqueous solution of borax and a mixture of Glauber's salt and common salt, and agitating further prior to tanning.

11. In the process of producing leather from pickled skins, the steps of agitating a quantity of such skins in an aqueous solution of Glauber's salt, sodium acetate and acetic acid for about 30 minutes at about 90° F., then adding to the bath an aqueous solution of borax and Glauber's salt, and agitating for a period of about 30 minutes prior to tanning.

12. In the process of producing leather from pickled skins, the steps of agitating a quantity of skins for about 30 minutes at 90° F. in a float of a composition of the following proportions: for 450 pounds of skins, 100 gallons of float containing 100-200 pounds Glauber's salt; about 40.5 pounds sodium acetate; and about 5.8 pounds acetic acid; then adding to the bath a solution of about 9.0 pounds borax in about 25 gallons of water with enough Glauber's salt to attain a salt concentration of about 15%; agitating for 30 minutes at approximately 80° F.; and draining the skins preparatory to tanning.

13. In the process of producing leather from pickled skins, the steps of agitating a quantity of such skins in an aqueous solution of Glauber's salt, sodium acetate and acetic acid such as to raise the pH number of the bath and skins to about 5.0-5.2, then adding to the bath an aqueous solution of borax and Glauber's salt, and agitating prior to tanning.

14. In the process of chrome tanning of skins which have been subjected to pickling in a strong acid, the steps of raising the pH number of pickled skins to the range of approximately 5.0-6.0 by replacement of the strong acid by acetic acid and maintaining approximately the same range of hydrogen ion concentration throughout the subsequent chrome tanning process.

15. In the process of chrome tanning of skins

which have been subjected to pickling in a strong acid, the steps of replacing the strong acid by a soluble fatty organic acid, adding small quantities of a neutralizing agent, and chrome tanning the skins.

16. In the process of chrome tanning of skins, which have been subjected to pickling in a strong acid, the steps of treating the pickled skins with a solution containing the salt of a soluble organic acid, whereby the strong acid is replaced by the weaker organic acid, and tanning the skins with a chrome solution.

17. In the process of chrome tanning of skins, which have been subjected to pickling in a strong acid, the steps of treating the pickled skins with a solution containing the salt of a soluble organic acid in the presence of a quantity of said organic acid itself, whereby the strong acid is replaced by the weaker organic acid, adding a small quantity of a neutralizing agent which will not alter the pH number appreciably, and tanning the skins with a chrome solution.

18. In the process of chrome tanning of skins, which have been subjected to pickling in a strong acid, the steps of agitating the pickled skins in a bath containing Glauber's salt, sodium acetate, and acetic acid; adding a solution of borax and Glauber's salt; agitating further; draining the skins; adding a salt solution and agitating while adding successive feeds of basic chromium sulphate until the skins are suitably tanned.

19. In the process of chrome tanning of skins, which have been subjected to pickling in a strong acid, the steps of agitating the pickled skins in a bath containing common salt, sodium acetate, and acetic acid; adding a solution of borax and common salt; agitating further; draining the skins; adding a salt solution and agitating while

adding successive feeds of basic chromium sulphate until the skins are suitably tanned.

20. In the production of leather from skins pickled in the strong acid of the pickle solution, the step comprising replacing the strong acid in said skins with a soluble fatty organic acid.

21. In the production of leather from skins pickled in strong acid, the step comprising reacting the strong acid in said skins with a soluble salt of an organic acid forming an organic acid soluble in water.

22. In the production of leather from skins pickled in strong acid, the steps comprising reacting the strong acid in said skins with a soluble salt of an organic acid and partially neutralizing the acid formed.

23. In the production of leather from raw skins pickled in strong acid, the steps comprising reacting strong acid in said skins with a salt of an organic acid in the presence of a quantity of the organic acid itself.

24. In the production of leather from skins pickled in strong acid, the steps comprising soaking said skins in a solution containing an alkali salt of an organic acid soluble in water, and, neutralizing the acid in the skins preparatory to converting the skins into leather.

25. In the process of producing leather from skins which have been pickled in a strong acid, the steps of replacing the strong acid in the skins with acetic acid prior to tanning.

26. In the production of leather from raw skins pickled in strong acid, the steps comprising reacting the strong acid in said skins with a salt of acetic acid in the presence of a quantity of acetic acid itself.

GEORGE R. PENSEL.